



US011594362B2

(12) **United States Patent**  
**Ochiai et al.**

(10) **Patent No.:** US 11,594,362 B2  
(45) **Date of Patent:** Feb. 28, 2023

(54) **CORE COMPONENT, METHOD OF MANUFACTURING SAME, AND INDUCTOR**

(71) Applicant: **KYOCERA Corporation**, Kyoto (JP)

(72) Inventors: **Hitomi Ochiai**, Omihachiman (JP); **Masamichi Shingu**, Shiga (JP); **Yuki Kitagawa**, Higashiomii (JP); **Hideki Mori**, Shiga (JP); **Mitsuya Takayama**, Koka (JP)

(73) Assignee: **KYOCERA Corporation**, Kyoto (JP)

(\*) Notice: Subject to any disclaimer, the term of this patent is extended or adjusted under 35 U.S.C. 154(b) by 786 days.

(21) Appl. No.: **16/524,769**

(22) Filed: **Jul. 29, 2019**

(65) **Prior Publication Data**

US 2020/0227196 A1 Jul. 16, 2020

(30) **Foreign Application Priority Data**

Jan. 11, 2019 (JP) ..... JP2019-003550

(51) **Int. Cl.**

**H01F 27/25** (2006.01)  
**H01F 27/255** (2006.01)  
**H01F 41/06** (2016.01)  
**H01F 41/02** (2006.01)  
**H01F 27/28** (2006.01)

(52) **U.S. Cl.**

CPC ..... **H01F 27/255** (2013.01); **H01F 27/2823** (2013.01); **H01F 41/0246** (2013.01); **H01F 41/06** (2013.01)

(58) **Field of Classification Search**

USPC ..... 336/221, 21, 83  
See application file for complete search history.

(56)

**References Cited**

**U.S. PATENT DOCUMENTS**

5,767,759 A \* 6/1998 Rouet ..... H01F 17/045  
336/212  
6,339,364 B1 \* 1/2002 Reddy ..... H03H 7/06  
336/212  
2016/0118183 A1 \* 4/2016 Wada ..... H01F 27/292  
336/192  
2016/0217919 A1 \* 7/2016 Iwata ..... H01F 27/29

(Continued)

**FOREIGN PATENT DOCUMENTS**

JP S59-166413 A 9/1984  
JP H05-275256 A 10/1993  
JP 2017-204596 A 11/2017

*Primary Examiner* — Tszfung J Chan

*Assistant Examiner* — Kazi S Hossain

(74) *Attorney, Agent, or Firm* — Procopio Cory Hargreaves and Savitch LLP

(57) **ABSTRACT**

A core component is made of a sintered body of an inorganic powder, in which the core component includes a columnar winding portion around which a conductive wire is wound, the columnar winding portion having a first axial end and a second axial end and a flange portion integrally formed with the winding portion at both axial ends of the winding portion, in which the columnar winding portion includes, in a cross section orthogonal to an axial center, a first region having a curved outer peripheral surface having a first radius of curvature and a second region having a curved surface having a second radius of curvature, the second radius of curvature is smaller than the first radius of curvature and the first region and the second region are connected with each other via a first projection.

**13 Claims, 5 Drawing Sheets**



(56)

**References Cited**

U.S. PATENT DOCUMENTS

- 2017/0169927 A1 \* 6/2017 Miyamoto ..... H01F 17/03  
2017/0330672 A1 11/2017 Uchida et al.  
2017/0330676 A1 \* 11/2017 Uchida ..... H01F 27/292

\* cited by examiner

FIG. 1A



FIG. 1B



FIG. 1C



FIG. 2 A



FIG. 2 B



FIG. 3 A



FIG. 3 B



FIG. 4 A



FIG. 4 B



FIG. 5 A (PRIOR ART)



FIG. 5 B (PRIOR ART)



## 1

CORE COMPONENT, METHOD OF  
MANUFACTURING SAME, AND INDUCTOR

## BACKGROUND OF THE INVENTION

## 1. Field of the Invention

The present disclosure relates to a core component made of a sintered body of an inorganic powder, a method of manufacturing the core component, and an inductor.

## 2. Description of Related Art

Conventionally, when winding a conductive wire, for example, a conductive wire covered with an insulating material such as polyurethane or polyester, around a winding portion of a core component such as a ferrite core, as shown in FIGS. 5A and 5B, a conductive wire 103 is mounted in a state of being aligned with a winding portion 101 by fixing the end of the conductive wire 103 to any one of a flange portion 102 provided at both ends of the winding portion 101 of a core component 100, and feeding the conductive wire 103 from one end to the other end of the winding portion 101 while bringing adjacent conductive wires 103 and 103 into contact with each other (Japanese Patent Application Laid-Open No. 5-275256). In FIG. 5A, reference numeral 104 is a lead-out electrode connecting both ends of the conductive wire 103.

Recently, as shown in Japanese Patent Application Laid-Open No. 2017-204596, the miniaturization of electronic devices such as portable terminals is progressing, and the demand for miniaturization of ferrite cores mounted on such electronic devices is also increasing. Further, Japanese Patent Application Laid-Open No. 2017-204596 discloses that the conductive wire which is wound around the winding portion is also thinned, and the diameter thereof is as thin as about 20  $\mu\text{m}$ .

Japanese Utility Model Laid-Open Publication No. 59-166413 proposes an inductance core having a columnar coil winding portion having a substantially elliptical cross section, and a pair of flanges each composed of substantially elliptical flat plate at both ends thereof.

## SUMMARY OF THE INVENTION

A core component of the present disclosure is made of a sintered body of an inorganic powder, in which the core component includes a columnar winding portion around which a conductive wire is wound, the columnar winding portion having a first axial end and a second axial end and a flange portion integrally formed with the columnar winding portion at both axial ends of the columnar winding portion, in which the columnar winding portion comprises, in a cross section orthogonal to an axial center, a first region including a curved outer peripheral surface having a first radius of curvature and a second region including a curved surface having a second radius of curvature, in which the second radius of curvature is smaller than the first radius of curvature, and the first region and the second region are connected with each other via a projection.

A method of manufacturing a core component according to the present disclosure includes filling and pressure molding an inorganic powder between an upper punch and a lower punch to form a pressure-molded compact, in which each of the upper punch and lower punch has an arc-shaped pressing surface for molding the columnar winding portion and the flange portion; and sintering the pressure-molded

## 2

compact, in which the arc-shaped pressing surface of the upper punch and the arc-shaped pressing surface of the lower punch have different radii of curvature, and the sintered compact is polished to form the projection at the boundary between the first region and the second region in the winding portion.

Another core component of the present disclosure is made of a sintered body of an inorganic powder, in which the core component includes a columnar winding portion around which a conductive wire is wound and a flange portion integrally formed with the winding portion at both axial ends of the winding portion, in which the flange portion includes, in a cross section orthogonal to an axial center, a third region having a curved outer peripheral surface having a large radius of curvature and a fourth region whose entire outer peripheral surface is composed of a curved surface having a small radius of curvature, or that has a flat portion whose outer peripheral surface is connected to the third region and a curved surface portion continuous with the flat portion and having a small radius of curvature, and the third region and the fourth region are connected with each other via a second projection.

Another method of manufacturing a core component according to the present disclosure includes filling and pressure molding an inorganic powder between an upper punch and a lower punch each of which has an arc-shaped pressing surface for forming the winding portion and the flange portion; and sintering the pressure-molded compact, in which the pressing surface of the upper punch and the pressing surface of the lower punch have different radii of curvature, and the sintered compact is polished to form the second projection at the boundary between the third region and the fourth region in the flange portion.

The inductor of the present disclosure includes the core component and a conductive wire wound around the winding portion of the core component.

## BRIEF DESCRIPTION OF THE DRAWINGS

FIG. 1A is a side view of a core component according to an embodiment of the present disclosure, and FIG. 1B is a sectional view thereof taken along line X-X, and FIG. 1C is a sectional view thereof taken along line Y-Y;

FIG. 2A and FIG. 2B are a cross-sectional view and a longitudinal-sectional view, respectively, showing how a core component according to an embodiment of the present disclosure is molded with a molding die;

FIG. 3A and FIG. 3B are respectively a cross-sectional view and a longitudinal-sectional view showing a state after molding with a molding die;

FIG. 4A is a partial enlarged cross-sectional view of the core component, and FIG. 4B is a partial enlarged cross-sectional view of another core component; and

FIG. 5A is a perspective view of a conventional core component around which a conductive wire is wound, and FIG. 5B is a longitudinal-sectional view thereof.

DETAILED DESCRIPTION OF PREFERRED  
EMBODIMENTS

Hereinafter, core components according to an embodiment of the present disclosure will be described. As shown in FIG. 1A, a core component 1 includes a columnar winding portion 2 having a first axial end and a second axial end and a flange portion 3 integrally formed with the winding portion 2 at both axial ends of the winding portion 2. The core component 1 is made of a sintered body of an

inorganic powder such as alumina in addition to ferrite. A conductive wire (not shown) is wound around the winding portion 2. Both ends of the conductive wire are connected to the lead-out electrodes formed on the flange portion 3. For example, the length in the axial direction of the winding portion 2 is 1 mm to 2 mm, and the diameter is 0.5 mm to 2 mm. Further, the length (width) of each flange portion 3 in the axial direction is 0.2 mm to 0.8 mm, and the diameter is 1.5 mm to 4 mm.

As shown in FIG. 1B and FIG. 4A described later, in the cross section orthogonal to the axial center, the winding portion 2 has a first region 11 having a curved outer peripheral surface having a first radius of curvature, and a second region 12 having a curved surface having a second radius of curvature. The second radius of curvature is smaller than the first radius of curvature. The first region 11 and the second region 12 are connected to each other via the projection 13. Therefore, disconnection of the conductive wire can be suppressed.

The projection 13 preferably has a curved outer peripheral surface. Further, the height of the projection 13 is preferably equal to or smaller than the diameter of the conductive wire in order to suppress the disconnection of the conductive wire. Here, the height of the projection 13 can be obtained by subtracting (the length from the axial center to the surface of the second region 12 including a second radius of curvature) from (the length from the axial center to the surface of the projection 13). In addition, in the case of the conductive wire provided with the coating, let the diameter of conductive wire be a diameter including a coating.

Furthermore, the outer peripheral surface of the projection 13 preferably has a radius of curvature smaller than that of the second radius of curvature of the winding portion 2. As a result, the residual stress in the projection 13 is reduced, so that the projection 13 is less likely to be brittlely fractured, and the occurrence of particle shedding due to the brittle fracture is reduced.

Alternatively, a stepped portion 10 may be largely removed by polishing or the like, and the portion may be processed into a planar shape. In this case, as shown in FIG. 4B, in the cross section orthogonal to the axial center, a winding portion 2' has a first region 11' having a curved outer peripheral surface having a first radius of curvature, and a second region 12' having a curved outer peripheral surface having the second radius of curvature and a flat portion 14 continuous with the curved outer peripheral surface. A second region 12' is connected to the first region 11' via a projection 13'.

As shown in FIG. 1C, in the cross section orthogonal to the axial center, the flange portion 3 has a first region 111 having a curved outer peripheral surface having a first radius of curvature, and a second region 112 including a curved surface portion having a curved surface having a second radius of curvature, and the first region 111 and the second region 112 are connected via a projection 131. As a result, it is possible to suppress the occurrence of particle shedding from the projection 131.

The projection 131 preferably has a curved outer peripheral surface. Furthermore, the outer peripheral surface of the projection 131 preferably has a radius of curvature smaller than that of the second radius of curvature of the flange portion. As a result, the residual stress in the projection 13 is reduced, so that the projection 13 is less likely to be brittlely fractured, and the occurrence of particle shedding due to the brittle fracture is reduced.

As in the winding portion 2 shown in FIG. 4B, the second region 112 may include the flat portion 14 which is con-

tinuous with a curved peripheral surface having the second radius of curvature and is connected to the first region 111 via the projection at the flat portion 14.

In the core component 1 of the present embodiment, as shown in FIG. 1B, when the winding portion 2 is observed in a cross section perpendicular to the axial direction, a surface layer portion 21 of the winding portion 2 has an area occupancy of voids smaller than that of an inside 22 of the winding portion 2. For example, the area occupancy of voids in the surface layer portion 21 of the winding portion 2 is 0.5 to 3%.

Therefore, since the surface layer portion 21 of the winding portion 2 is dense, the conductive wire can be wound around the winding portion 2 with high accuracy, the strength of the winding portion 2 is improved, the resistance to deformation is improved, and particle shedding is also suppressed.

Here, the surface layer portion 21 refers to a region having a depth of 0.22 mm or less from the surface of the winding portion 2 toward the axial center. The inside 22 refers to a region excluding the surface layer portion 21. Further, in order to obtain the area occupancy of voids, for example, the portion where the size and distribution of the voids are observed on average is selected among the mirror surface of each of the surface layer portion 21 and the inside 22 obtained by polishing them using diamond abrasive grains having an average particle diameter of 1  $\mu\text{m}$  (this mirror surface is the cross section perpendicular to the axial direction of the winding portion 2). For example, the range in which the area is  $3.84 \times 10^{-2} \text{ mm}^2$  (lateral length is 0.226 mm, longitudinal length is 0.170 mm) is photographed with a scanning electron microscope at a magnification of 500 to obtain an observation image. Then, for this observation image, the area occupancy of voids can be determined by a method called the particle analysis using the image analysis software "A-Zou Kun (ver 2.52)" (registered trademark, manufactured by Asahi Kasei Engineering Corporation, in the following description, the description of the image analysis software "A-Zou Kun" refers to the image analysis software manufactured by Asahi Kasei Engineering Corporation).

The area occupancy of voids of the flange portion 3 may have the same relationship as that of the winding portion 2. That is, as shown in FIG. 1C, when the flange portion 3 is observed in a cross section perpendicular to the axial direction, the surface layer portion of the flange portion 3 has an area occupancy of voids smaller than an area occupancy of voids of an inside 32 of the flange portion 3. For example, the area occupancy of voids in a surface layer portion 31 of the flange portion 3 is 0.5 to 4%.

In addition, it is preferable that a gap C between adjacent voids represented by the following Formula at least in the surface layer portion 21 of the winding portion 2 be 6 to 12  $\mu\text{m}$ .

$$\text{Formula: } C = L - R$$

where, L is the average value of the distance between the centers of gravity between adjacent voids in the surface layer portion 21 or the inside 22, and R is the average value of the equivalent circle diameters of the voids in the surface layer portion 21 or the inside 22.

At this time, it is more preferable that the voids present in the surface layer portion 21 have a larger gap C between adjacent voids than the voids present in the inside 22. Specifically, it is preferable that the difference between the gap  $C_{S1}$  between the voids in the surface layer portion 21 and

the gap  $C_{S2}$  between the voids in the inside 22 obtained from the above formula be 1  $\mu\text{m}$  or more.

As described above, since the void distribution at least in the surface layer portion 21 of the winding portion 2 is sparse, so that the particle shedding generated from the inside and the outline of the voids is reduced, and when the conductive wire is wound around the winding portion 2, it is not likely to cause damage to the conductive wire such as disconnection.

As in the winding portion 2, the voids present in the surface layer portion 31 of the flange portion 3 may have a larger gap  $C$  between adjacent voids shown by the above formula than the voids present in the inside 32. Specifically, the difference between the gap  $C_{F1}$  between the voids in the surface layer portion 31 and the gap  $C_{F2}$  between the voids in the inside 32 is 1  $\mu\text{m}$  or more. Here, the surface layer portion 31 refers to a region having a depth of 0.22 mm or less from the surface of the flange portion 3 toward the axial center. The inside 32 refers to a region excluding the surface layer portion 31.

The average value of the distance between the centers of gravity between the voids and the average value of the equivalent circle diameters of the voids can be determined by the following method.

First, the portion where the size and distribution of the voids are observed on average is selected among the mirror surface of each of the surface layer portion and the inside obtained by polishing them using diamond abrasive grains (this mirror surface is the cross section perpendicular to the axial direction of the winding portion 2). For example, the range in which the area is  $3.84 \times 10^{-2} \text{ mm}^2$  (lateral length is 0.226 mm, longitudinal length is 0.170 mm) is photographed with a scanning electron microscope at a magnification of 500 to obtain an observation image. Next, using the above-mentioned image analysis software "A-Zou Kun", the average value of the distances between the centers of gravity of the voids can be determined by the distance-between-centroid method of dispersion measurement.

In addition, the average value of the equivalent circle diameters of the voids can be determined by performing analysis using the same observation image as the above-described observation image by means of the particle analysis using the image analysis software "A-Zou Kun".

As the setting conditions of the distance-between-centroid method and the particle analysis, for example, a threshold value which is an index indicating light and dark of an image may be 83, lightness may be dark, a small figure removing area may be 0.2  $\mu\text{m}^2$  and a noise removing filter may be present. In the above measurement, the threshold value is 83, but the threshold value may be adjusted according to the brightness of the observation image. The lightness is dark, the method of binarization is manual, and the small figure removing area is 0.2  $\mu\text{m}^2$  and a noise removing filter is present. The threshold value may be adjusted so that a marker whose size changes according to the threshold value in the observation image matches the shape of the voids.

The winding portion 2 preferably has a cutting level difference ( $R\delta c$ ) of the surface roughness curve of 0.2  $\mu\text{m}$  or more and 2  $\mu\text{m}$  or less. The cutting level difference ( $R\delta c$ ) represents the difference between the cutting level at a 25% loading length rate in the surface roughness curve and the cutting level at a 75% loading length rate in the roughness curve. The cutting level difference ( $R\delta c$ ) is a parameter that represents both the axial direction and the radial direction.

Similarly, the cutting level difference  $R\delta c$  of the roughness curve on the surface of the flange portion 3 is preferably 0.2  $\mu\text{m}$  or more and 2  $\mu\text{m}$  or less.

When the cutting level difference ( $R\delta c$ ) is 0.2  $\mu\text{m}$  or more, an appropriate anchor effect can be given to the conductive wire. Therefore, the slip of the conductive wire is appropriately suppressed, the winding installation becomes easy, and the winding of the conductive wire to the winding portion 2 can be performed with high accuracy, so that the occurrence of winding deviation or the like can be prevented. On the other hand, the cutting level difference ( $R\delta c$ ) is 2  $\mu\text{m}$  or less, so that it is possible to suppress the variation in the intervals between the wound conductive wires and the height difference between the adjacent conductive wires.

Moreover, it is preferable that the root mean square height ( $Rq$ ) in a roughness curve be 0.07  $\mu\text{m}$  or more and 2.5  $\mu\text{m}$  or less.

When the root mean square height ( $Rq$ ) is 0.07  $\mu\text{m}$  or more, an appropriate anchor effect can be given to the conductive wire, which facilitates the mounting. On the other hand, when the conductive wire is wound with a root mean square height ( $Rq$ ) of 2.5  $\mu\text{m}$  or less, the risk of disconnection can be reduced.

The winding portion 2 is pressure-molded at a high pressure by a lower punch 5 and an upper punch 6 as described later, so that the surface layer portion 21 of the winding portion 2 is denser than a surface layer portion 31' of an inner portion of the flange portion 3 shown in FIG. 1A. Therefore, when the conductive wire is wound, it is possible to reduce the risk of particle shedding caused by the winding.

The cutting level difference  $R\delta c$  and the root mean square height ( $Rq$ ) of the roughness curve are in accordance with JIS B 0601: 2001, and can be measured by a ultra-depth color 3D shape measuring microscopes (for example, VK-9500 manufactured by Keyence Corporation). The measurement conditions are as follows; measurement mode: color ultra depth, gain: 953, measurement resolution in the height direction (pitch): 0.05  $\mu\text{m}$ , magnification: 400 times, cutoff value  $\lambda_s$ : 2.5  $\mu\text{m}$ , cutoff value  $\lambda_c$ : 0.08 mm.

Here, it is sufficient that the measurement range per one location is 580  $\mu\text{m}$  to 700  $\mu\text{m} \times 280 \mu\text{m}$  to 380  $\mu\text{m}$  when the winding portion 2 is to be measured, and 70  $\mu\text{m}$  to 170  $\mu\text{m} \times 500 \mu\text{m}$  to 550  $\mu\text{m}$  when the flange portion 3 is to be measured.

As shown in FIG. 1A, the radius of curvature of a corner portion 20 where the winding portion 2 and the flange portion 3 intersect is preferably equal to or smaller than the diameter of the conductive wire. Specifically, the radius of curvature of the corner portion 20 is 40  $\mu\text{m}$  or less, preferably 10 to 30  $\mu\text{m}$ .

As a result, the occurrence of offset at the corner portion can be suppressed, and the conductive wire can be accurately wound in a state of being aligned with the winding portion.

Next, a method of manufacturing the core component 1 by press molding will be described based on FIGS. 2 and 3. FIGS. 2A and 2B are a cross-sectional view and a longitudinal-sectional view, respectively, showing the molding state of the core component 1. The press molding apparatus used includes a die 4, the lower punch 5 and the upper punch 6. The lower punch 5 includes a first lower punch 51 and a second lower punch 52. The upper punch 6 includes a first upper punch 61 and a second upper punch 62.

As shown in FIG. 2A, the lower punch 5 and the upper punch 6 have arc-shaped pressing surfaces 50a, 50b, 60a, and 60b for forming the winding portion 2 and the flange portion 3, respectively. The radii of curvature of the pressing surfaces 50a and 50b of the lower punch 5 and the pressing surfaces 60a and 60b of the upper punch 6 at the

portion forming the winding portion 2 and the flange portion 3 are different. In this embodiment, the radius of curvature of the pressing surfaces 60a and 60b of the upper punch 6 is formed larger than the radius of curvature of the pressing surfaces 50a and 50b of the lower punch 5. Conversely, the radius of curvature of the pressing surfaces 50a and 50b of the lower punch 5 may be larger than the radius of curvature of the pressing surfaces 60a and 60b of the upper punch 6.

Therefore, stepped portions 7 and 7' are formed on both sides in a state where the pressing surfaces 50a and 50b of the lower punch 5 and the pressing surfaces 60a and 60b of the upper punch 6 overlap with each other.

In the present embodiment, at least the radius of curvature of the pressing surface 50b of the lower punch 5 and the radius of curvature of the pressing surface 60b of the upper punch 6 may be different from each other at a portion where the winding portion 2 is to be formed.

In molding, first, the lower punch 5 is fixed in the die 4 as shown in FIG. 2A, and an inorganic powder 8 as the raw material is supplied to the pressing surfaces 50a and 50b of the upper surface of the lower punch 5. Then, the upper punch 6 is lowered to press the inorganic powder between the lower punch 5 and the upper punch 6.

The molding pressure at the time of pressure molding is 98 MPa or more, preferably 196 to 490 MPa. Since such a high pressure can be used for pressure molding, the resulting compact has a high density and is closely packed especially on the surface portion, and faithfully reflects the surface shape of the molding die (lower punch 5 and upper punch 6 described later), so that the radius of curvature of the corner portion 20 where the winding portion 2 and the flange portion 3 intersect can be equal to or smaller than the diameter of the conductive wire.

Further, as described above, the area occupancy of voids of the surface layer portion 21 of the winding portion 2 can be made smaller than that of the inside 22 of the winding portion.

For the same reason, the void distribution at least in the surface layer portion 21 of the winding portion 2 can be made sparse, and the gap C between adjacent voids can be made 6 to 12  $\mu\text{m}$ .

In addition, the compact has a dense and closely packed surface, in particular, on the surface portion, so that the cutting level difference  $R_{\text{dc}}$  of the roughness curve of the surface of the winding portion 2 can be 0.2 to 2  $\mu\text{m}$ .

Such high pressure can be applied because, as described above, the pressing surfaces 50a and 50b of the lower punch 5 and the pressing surfaces 60a and 60b of the upper punch 6 have different radii of curvature. On the other hand, when the pressing surfaces 50a and 50b of the lower punch 5 and the pressing surfaces 60a and 60b of the upper punch 6 have the same radius of curvature, the compact cannot be taken out of the molding die when pressurized with high pressure. Therefore, since it cannot be pressurized at high pressure but must be pressurized at low pressure, the core component 1 formed by pressure molding has a lot of voids, the strength is inferior, and further, it is easy to generate the particle shedding.

After molding, as shown in FIGS. 3A and 3B, the die 4 is lowered relative to the lower punch 5 and the upper punch 6 so that the stepped portions 7 and 7' and the upper end face of the die 4 on the overlapping surface of the lower punch 5 and the upper punch 6 have approximately the same height. Next, the upper punch 6 is moved upward relative to the lower punch 5. At this time, first, the first upper punch

61 on both sides is raised, and then the second upper punch 62 is raised. This facilitates separation of the upper punch 6 from the compact 9.

The second lower punch 52 is relatively raised with respect to the die 4 simultaneously with or after the rise of the upper punch 6. As a result, the compact 9 can be pushed up, and the compact 9 can be easily taken out.

After removing the raw material powder adhering to the obtained compact 9 by air blow or the like if necessary, for example, the compact 9 is held at the maximum temperature of 1000 to 1200°C. for 2 to 5 hours in an air atmosphere to obtain the sintered body. Further, the sintered body is subjected to polishing such as barrel polishing, if necessary, to obtain the core component 1.

Stepped portions 10 and 10' corresponding to the stepped portions 7 and 7' due to the difference in the radii of curvature of the pressing surfaces 50a and 50b of the lower punch 5 and the pressing surfaces 60a and 60b of the upper punch 6 is formed on the surface of the compact 9 corresponding to the winding portion 2 and the flange portion 3. If the stepped portions 10 and 10' have a problem in winding the conductive wire around the surface of the winding portion 2, it is preferable to remove as much as possible by polishing.

As shown in FIG. 4A, for the core component 1 obtained by polishing, the winding portion 2 has a first region 11 having a curved outer peripheral surface with a large radius of curvature and a second region 12 having a curved outer peripheral surface with a small radius of curvature in a cross section orthogonal to the axial center, and the first region 11 and the second region 12 are connected via a projection 13. At this time, the height of the projection 13 is preferably equal to or smaller than the diameter of the conductive wire wound around the outer peripheral surface of the winding portion 2. As a result, the occurrence of disconnection and offset of the conductive wire can be suppressed.

In addition, the stepped portions 10 and 10' may be largely removed by polishing, and the portion may be processed into a planar shape. In this case, as shown in FIG. 4B, in the cross section orthogonal to the axial center, a winding portion 2' has a first region 11' having a curved outer peripheral surface with a large radius of curvature, and a second region 12' consisting of a flat portion 14 whose outer peripheral surface is connected to the first region 11' and a curved surface portion continuous with the flat portion 14 with a small radius of curvature, and the first region 11' and the second region 12' are connected via a projection 13'.

The above polishing process may be applied not only to the winding portions 2 and 2' but also to the flange portion 3 in the same manner.

The obtained core component 1 is suitably used as an inductor by winding a conductive wire around the winding portions 2 and 2'. The application of the core component 1 of the present disclosure is not limited to the inductor, and may be applied to the case where members having flanges at both ends and a central portion having a columnar shape and a smooth curved surface shape are formed of ceramics or the like. For example, in the case of manufacturing, with a ceramic, a tape guide for guiding a magnetic tape or the like, in which the tape guide has flanges at both ends of a columnar body, the manufacturing can be easily performed by using the core component manufacturing method of the present disclosure.

What is claimed is:

1. A core component made of a sintered body of an inorganic powder, the core component comprising:

a columnar winding portion around which a conductive wire is wound, the columnar winding portion having a first axial end and a second axial end;  
 a flange portion integrally formed with the columnar winding portion at both axial ends of the columnar winding portion,  
 wherein the columnar winding portion comprises, in a cross section orthogonal to an axial center, a first region including a curved outer peripheral surface having a first radius of curvature and a second region including a curved surface having a second radius of curvature, wherein the second radius of curvature is smaller than the first radius of curvature, and  
 the first region and the second region are connected with each other via a projection.

2. The core component according to claim 1, wherein the second region further includes a flat portion which continues with the curved outer peripheral surface having the second radius of curvature, and the second region is connected to the first region via the projection at the flat portion.

3. The core component according to claim 1, wherein a height of the projection is equal to or smaller than a diameter of the conductive wire.

4. The core component according to claim 1, wherein the projection has a curved outer peripheral surface.

5. The core component according to claim 4, wherein a radius of curvature of the curved outer peripheral surface of the projection is smaller than the second radius of curvature of the columnar winding portion.

6. A core component made of a sintered body of an inorganic powder, the core component comprising:

a columnar winding portion around which a conductive wire is wound, the columnar winding portion having a first axial end and a second axial end;  
 a flange portion integrally formed with the columnar winding portion at both axial ends of the columnar winding portion,  
 wherein the flange portion includes, in a cross section orthogonal to an axial center, a first region including a curved outer peripheral surface having a first radius of curvature and a second region including a curved surface having a second radius of curvature, wherein the second radius of curvature is smaller than the first radius of curvature, and  
 the first region and the second region are connected with each other via a projection.

7. The core component according to claim 6, wherein the second region further includes a flat portion which continues

with the curved outer peripheral surface having the second radius of curvature, and the second region is connected to the first region via the projection at the flat portion.

8. The core component according to claim 6, wherein the projection has a curved outer peripheral surface.

9. The core component according to claim 8, wherein a radius of curvature of the curved outer peripheral surface of the projection is smaller than the second radius of curvature of the flange portion.

10. A method of manufacturing the core component according to claim 1, the method comprising:

filling and pressure molding an inorganic powder between an upper punch and a lower punch to form a pressure-molded compact, wherein each of the upper punch and lower punch has an arc-shaped pressing surface for forming the columnar winding portion and the flange portion; and  
 sintering the pressure-molded compact to form a sintered body,

wherein the arc-shaped pressing surface of the upper punch and the arc-shaped pressing surface of the lower punch have different radiiuses of curvature, and  
 polishing the sintered body to form the first projection at a boundary between the first region and the second region in the columnar winding portion.

11. A method of manufacturing the core component according to claim 6, the method comprising:

filling and pressure molding an inorganic powder between an upper punch and a lower punch to form a pressure-molded compact, wherein each of the upper punch and lower punch has an arc-shaped pressing surface for forming the columnar winding portion and the flange portion; and  
 sintering the pressure-molded compact to form a sintered body,

wherein the arc-shaped pressing surface of the upper punch and the arc-shaped pressing surface of the lower punch have different radiiuses of curvature, and  
 polishing the sintered body to form the first projection at a boundary between the first region and the second region in the flange portion.

12. An inductor comprising the core component according to claim 1 and a conductive wire wound around a winding portion of the core component.

13. An inductor comprising the core component according to claim 6 and a conductive wire wound around a winding portion of the core component.

\* \* \* \* \*